

1

3,328,419

**COLOUR COUPLERS AND THEIR PRODUCTION  
AND USE IN COLOUR PHOTOGRAPHY**

Brian Anderson, Marple, England, assignor to Ilford Limited, Essex, England, a British company

No Drawing. Filed June 15, 1964, Ser. No. 375,308  
Claims priority, application Great Britain, June 17, 1963,

24,027/63

6 Claims. (Cl. 260—310)

This invention relates to colour couplers and to their production and use in colour photography.

Many modern processes of colour photography are based on the development of a developable silver salt photographic image by means of an aromatic primary amino compound, such as an N,N-diethyl p-phenylene diamine or a derivative thereof in the presence of a so-called colour coupler, this being a compound which will couple with the oxidation products of the developer to yield a dye image, usually an azamethine or quinone-imine dye image, in situ with the developed silver.

Where, as in many of the processes, the colour coupler is incorporated in the photographic emulsion layer in which the image is ultimately to be formed, it is important that it should be non-diffusing in such layer, i.e. that it should neither diffuse away during the processing steps nor migrate from its layer to any adjacent layer. Many attempts have been made to achieve this characteristic of non-diffusibility, i.e. to make the colour coupler substantive to the medium, usually gelatin, of the photographic emulsion. The methods which have been employed consist generally in the use of colour couplers containing groups of substantial molecular size, e.g. long chain alkyl groups, and also solubilising groups. Such colour couplers are often manufactured by a synthesis in which the group conferring non-diffusion and the solubilising group are introduced at separate stages and the colour couplers are often difficult to isolate and purify. It is one object of the present invention to provide a new class of colour couplers which are non-diffusing in photographic emulsion layers, and which may be manufactured by a simple synthetic process in which two solubilising groups and a group conferring non-diffusion are introduced simultaneously, and further the carboxylic acid group may be obtained in a protected form if so desired.

According to a first feature of the present invention there is provided, as a new class of colour couplers, compounds of the general Formula I



where the COOH group is ortho to the carbonylamino group, and the corresponding cyclised compounds of the general Formula II



where A is a grouping selected from the groups



B is a colour coupler residue as hereinafter defined, and R is an alkyl, aralkyl, cycloalkyl or aryl group.

By the term "colour coupler residue" used to define the symbol B is meant a grouping such that the compound B-H (and therefore also the compound B.NH<sub>2</sub>) is a compound which will react with the oxidation products of N,N-diethyl p-phenylene diamine, formed during the de-

2

velopment of a silver salt image with that compound, to yield a quinone-imine or azamethine dyestuff.

According to a further feature of the invention colour couplers of the foregoing general Formulas I and II are prepared by condensing a compound of the general Formula III



III

with a colour coupler of the general formula B-NH<sub>2</sub> where B has the meaning assigned to it above. A compound of the general Formula II is obtained if the ring structure of the compound of Formula III is retained; otherwise, if the ring opens, a product of Formula I is obtained.

The colour couplers containing an amino group which may be used in the process of the invention are for example:

(1) Those which contain a —COCH<sub>2</sub>CO— group, for example benzoyl-4-amino-2-methoxyacetanilide, 4'-methoxybenzoylacet-4-amino-2-methoxyanilide, the 2-alkoxybenzoylacet-amino-anilides described in British patent specification No. 595,314 or the aminobenzoylacet-methoxy-anilides of British patent specification No. 800,108, and which give yellow dyestuffs on colour development with substituted p-phenylene diamines.

(2) Those which contain a cyanacetyl group or a pyrazolone ring for example 4-*ω*-cyanacetylaniline, 1-methyl-3-amino-5-pyrazolone, 1-(*β*-hydroxyethyl)-3-amino-5-pyrazolone, 1-phenyl-3-amino-5-pyrazolone and substituted 1-aryl-3-amino-5-pyrazolones as described in British patent specification Nos. 547,064; 680,474; 680,488, the 1-heterocycle-3-amino-5-pyrazolones as described in British patent specification No. 599,919, the 1-(aminoaryl)-3-coumarilylamino-5-pyrazolones of British patent specification No. 890,305, the 1-alkyl-3-(aminophenoxyacetamido)-5-pyrazolones of British patent specification No. 865,720 or the 1-phenyl-3-amino-arylarnino-5-pyrazolones described in British patent specification No. 956,261 and which give magenta dyestuffs on colour development with substituted p-phenylene diamines.

(3) Phenols and 1-naphthols, which contain an amino group, for example 4-chloro-5-methyl-2-aminophenol or the aminophenols described in British patent specification Nos. 797,141; 754,306; 1-amino-5-naphthol, N(*β*-aminoethyl)-1-hydroxy-2-naphthamide or similar N-substituted naphthamides containing an amino group, as described in British patent specification No. 902,266 which may also be substituted in the 4-position, as described in British patent specification No. 757,368 and which give cyan dyestuffs on colour development with substituted p-phenylene diamines.

The new colour couplers of the invention may be used in the developing solution or they may be included in a light-sensitive layer or in a non-light-sensitive layer adjacent to a sensitive layer or separated therefrom by a water-permeable colloid layer.

It is a preferred feature of the invention to include the new colour couplers of the invention in a light-sensitive gelatino or gelatino-substitute silver halide emulsion layer which forms part of a multilayer film or paper of the kind used for colour photography.

The multilayer colour photographic material may be a natural order material in which the images are to be formed in colours complementary to those of the original object or one in which an unnatural order is used, for example one in which in the top layer there is formed a yellow image of the blue parts of the object, in one of the two layers there is formed a cyan image of the green parts of the object and in the other a magenta image of the red parts of the object.

The new colour couplers may be incorporated in the photographic emulsion layers by taking them up in dilute alkali, e.g. dilute sodium hydroxide, and adding the resulting solution to the emulsion. If a colour coupler of Formula II is used the alkali may cause the ring structure to break down yielding a product of Formula I.

Alternatively, the compounds may be dispersed, in a non-solvent medium, and the dispersion added to a photographic emulsion. Since in this case alkali is not used the products of Formula II remain with their ring structure intact, though they are possibly broken down by the effect of treatment of the emulsions with alkaline developers.

It is to be observed that in the compounds of Formula II the potential solubilising groups are protected in the form of the ring structure, so that the compounds are more readily isolated and purified. Nevertheless, the solubilising groups are freed as the compounds are dissolved in alkali for addition to the photographic emulsion.

The following examples will serve to illustrate the invention:

#### EXAMPLE 1

2-carboxy-N-(1-phenyl-5-pyrazolonyl-3)-benzamide-4-N'-(4-dodecylphenyl)-sulphonamide



A mixture of 11.75 parts of phthalic anhydride-4-N-(4-dodecylphenyl) sulphonamide, 4.35 parts of 1-phenyl-3-amino-5-pyrazolone and 110 parts of ethyl acetate is heated under reflux for 2 hours. 200 parts of 60-80 grade petroleum ether are then added and the precipitate obtained is filtered off, dried and recrystallised from 240 parts of methanol. The 8.5 parts of 2-carboxy-N-(1-phenyl-5-pyrazolonyl-3)-benzamide-4-N'-(4-dodecylphenyl) sulphonamide are obtained as a colourless solid

chloride obtained is removed by filtration. The solution is then evaporated to dryness in vacuo and the residue dissolved in 200 parts of water by the addition of 2 N sodium hydroxide solution. After filtering, the solution obtained is acidified with 2 N hydrochloric acid to precipitate the product which is collected by filtration and dried. The 7.1 parts of phthalic acid-4-N-(4-dodecylphenyl) sulphonamide are obtained as a colourless solid melting at 164-165° C. On analysis the compound is found to contain 64.0% of carbon, 7.0% of hydrogen, 3.1% of nitrogen and 6.7% of sulphur. ( $C_{26}H_{35}NO_6S$  requires 63.8% of carbon, 7.2% of hydrogen, 2.9% of nitrogen and 6.5% of sulphur.)

A photographic layer containing the colour coupler may be obtained in the following manner:

A mixture of 1.54 parts of the colour coupler and 12 parts of n-propyl alcohol is warmed to dissolve and 2.35 parts of 2 N potassium hydroxide then added. The solution so obtained is diluted to 30 parts with distilled water and added to 500 parts of a green sensitised gelatino silver halide emulsion containing silver halide equivalent to 2.5 parts of silver and 3.5% gelatin. The emulsion is then coated on film base and the coated layer dried. When the photographic material so obtained is exposed to green

light, developed in a colour developer containing 4-amino-N-ethyl-N- $\epsilon$ -hydroxypentylaniline, bleached and fixed, a magneta image is obtained which has an absorption maximum at a wavelength of light of 540 millimicrons.

#### EXAMPLE 2

2-carboxy - N - [3-(4-methoxybenzoylacetamide)-4-methoxyphenyl]benzamide - 4 - N' - (4-dodecylphenyl) sulphonamide



melting at 160-162° C. On analysis the compound is found to contain 64.3% of carbon, 6.0% of hydrogen, 8.4% of nitrogen and 4.4% of sulphur.



requires 64.3% of carbon, 6.8% of hydrogen, 8.35% of nitrogen and 4.4% of sulphur.)

The phthalic anhydride-4-N-(4-dodecylphenyl) sulphonamide used in the above example may be prepared as follows:

A mixture of 30 parts of phthalic acid-4-N-(4-dodecylphenyl)-sulphonamide and 300 parts of acetyl chloride is heated under reflux for 1 hour then evaporated to dryness in vacuo.

The solid residue is recrystallised from 400 parts of 60-80 grade petroleum ether. The 12.5 parts of phthalic anhydride-4-N-(4-dodecylphenyl) sulphonamide are obtained as a colourless crystalline solid melting at 83° C. On analysis the compound is found to contain 66.3% of carbon, 7.0% of hydrogen, 3.1% of nitrogen and 6.8% of sulphur. ( $C_{26}H_{35}NO_5S$  requires 66.3% of carbon, 7.0% of hydrogen, 3.0% of nitrogen and 6.8% of sulphur.)

The phthalic acid-4-N-(4-dodecylphenyl) sulphonamide itself may be prepared as follows:

A mixture of 5.3 parts of phthalic acid-4-sulphon chloride, 10.44 parts of p-dodecylaniline and 100 parts of ethyl acetate is heated under reflux for 12 hours, cooled to 20° C. and the precipitate of p-dodecylaniline hydro-

50 parts of ethyl acetate is heated at 50° C. for 1 hour, 500 parts of 60-80 grade petroleum ether are then added and the precipitate obtained filtered off, dried and recrystallised from 120 parts of methanol.

The 8.0 parts of 2-carboxy-N-[3-(4-methoxybenzoylacetamido)-4-methoxyphenyl]benzamide-4-N'-(4-dodecylphenyl)sulphonamide are obtained as a colourless solid melting at 135-137° C. On analysis the compound is found to contain 64.4% of carbon, 6.5% of hydrogen, 5.1% of nitrogen and 3.7% of sulphur.



60 requires 64.6% of carbon, 6.6% of hydrogen, 5.1% of nitrogen and 3.9% of sulphur.)

65 A photographic layer containing the colour coupler may be obtained in the following manner:

A mixture of 3.8 parts of the colour coupler and 20 parts of n-propyl alcohol is warmed to dissolve and 3.5 parts of 2 N potassium hydroxide solution then added. The solution so obtained is diluted to 70 parts with distilled water and added to 500 parts of a blue sensitised gelatino silver halide emulsion containing silver halide equivalent to 7.0 parts of silver and 4% gelatin. The emulsion is then coated on film base and the coated layer dried. When the photographic material so obtained is exposed to blue light, developed in a colour developer containing

4-amino-N-ethyl-N- $\epsilon$ -hydroxypentylaniline, bleached and fixed, a yellow image is obtained which has an absorption maximum at a wavelength of light of 440 millimicrons.

## EXAMPLE 3

2-carboxy-N-[ $\beta$ (1-hydroxy-2-naphthamido)ethyl]benzamide-4-N'-(4-dodecylphenyl)sulphonamide



A mixture of 8.05 parts of N-( $\beta$ -aminoethyl)-1-hydroxy-2-naphthamide, 16.45 parts of phthalic anhydride-4-N-(4-dodecylphenyl)-sulphonamide and 160 parts of ethyl acetate is heated at 50° C. for 1 hour and then allowed to stand until the product crystallises out. The 10.5 parts of 2-carboxy-N-[ $\beta$ (1-hydroxy-2-naphthamido)ethyl]benzamide-4-N'-(4-dodecylphenyl)sulphonamide are obtained as a colourless solid melting at 178-179° C. On analysis the compound is found to contain 66.9% of carbon, 6.6% of hydrogen, 6.1% of nitrogen and 4.5% of sulphur. (C<sub>39</sub>H<sub>47</sub>N<sub>3</sub>O<sub>7</sub>S requires 66.9% of carbon, 6.7% of hydrogen, 6.0% of nitrogen and 4.6% of sulphur.)

A photographic layer containing the colour coupler may be obtained in the following manner:

In place of the 8.05 parts of N-( $\beta$ -aminoethyl)-1-hydroxy-2-naphthamide used in Example 3 there are used 12.95 parts of 4-aminobenzoylacet-(3:5-di-carbomethoxy)anilide. The product is obtained by evaporating the reaction mixture to dryness and crystallising the residue from methyl alcohol. The 3.5 parts of 2-carboxy-N-4-[3:5-di-carbomethoxyphenylaminocarbonyl]acetyl]phenylbenzamide-4-N'-(4-dodecylphenyl)sulphonamide are obtained as a solid melting at 128-131° C.

## EXAMPLE 4

2-carboxy-N-[4-(4-methoxybenzoylacetamido)-2:5-diethoxyphenyl]benzamide-4-N'-(4-dodecylphenyl)sulphonamide

35



A mixture of 2.53 parts of the colour coupler, 12 parts of n-propyl alcohol and 3.6 parts of 2 N potassium hydroxide solution is warmed to dissolve and then diluted to 40 parts with distilled water. The solution so obtained is added to 500 parts of a red sensitised gelatino silver halide emulsion containing silver halide equivalent to 2.0 parts of silver and 3.5% gelatin. The emulsion is then coated on a paper base and the coated layer dried. When the photographic layer so obtained is exposed to red light, developed in a colour developer containing 4-amino-N-ethyl-N- $\epsilon$ -hydroxypentylaniline, bleached and fixed, a cyan image is obtained.

## EXAMPLE 4

2-carboxy-N-[ $\beta$ (4-chlor-1-hydroxy-2-naphthamido)ethyl]benzamide-4-N'-(4-dodecylphenyl)sulphonamide



In place of the 8.05 parts of N-( $\beta$ -aminoethyl)-1-hydroxy-2-naphthamide used in Example 3, there are used 9.26 parts of N-( $\beta$ -aminoethyl)-4-chlor-1-hydroxy-2-naphthamide. The 6.5 parts of 2-carboxy-N-[ $\beta$ (4-chlor-1-hydroxy-2-naphthamido)ethyl]benzamide-4-N'-(4-dodecylphenyl)sulphonamide are obtained as a colourless solid melting at 203-204° C. and on analysis is found to contain 64.0% of carbon, 6.0% of hydrogen and 5.5% of

70 gen at 70-80° C. under a pressure of 100 atmospheres for 15 hours. After cooling the product is filtered off and recrystallised from ethyl alcohol. The 28 parts of 4-(4-methoxybenzoylacetamido)-2:5-diethoxyaniline are obtained as fawn needle crystals melting at 154-155° C.

The 4-(4-methoxybenzoylacetamido)-2:5-diethoxynitrobenzene itself may be prepared as follows:

nitrogen. (C<sub>39</sub>H<sub>46</sub>N<sub>3</sub>O<sub>7</sub>SCl requires 63.7% of carbon, 6.3% of hydrogen and 5.7% of nitrogen.)

## EXAMPLE 5

5 2-carboxy-N-4-(3:5-di-carbomethoxyphenylaminocarbonyl)acetyl]phenylbenzamide-4-N'-(4-dodecylphenyl)sulphonamide

In place of the 8.05 parts of N-( $\beta$ -aminoethyl)-1-hydroxy-2-naphthamide used in Example 3 there are used 12.95 parts of 4-aminobenzoylacet-(3:5-di-carbomethoxy)anilide. The product is obtained by evaporating the reaction mixture to dryness and crystallising the residue from methyl alcohol. The 3.5 parts of 2-carboxy-N-4-[3:5-di-carbomethoxyphenylaminocarbonyl]acetyl]phenylbenzamide-4-N'-(4-dodecylphenyl)sulphonamide are obtained as a solid melting at 128-131° C.

## EXAMPLE 6

2-carboxy-N-[4-(4-methoxybenzoylacetamido)-2:5-diethoxyphenyl]benzamide-4-N'-(4-dodecylphenyl)sulphonamide

35



In place of the 8.05 parts of N-( $\beta$ -aminoethyl)-1-hydroxy-2-naphthamide used in Example 3 there are used 13.02 parts of 4-(4-methoxybenzoylacetamido)-2:5-diethoxyaniline. The product is obtained by evaporating the reaction mixture to dryness in vacuo and recrystallising the residue from methanol. The 8.4 parts of 2-carboxy-N-[4-(4-methoxybenzoylacetamido)-2:5-diethoxyphenyl]benzamide-4-N'-(4-dodecylphenyl)sulphonamide are obtained as a solid melting at 94-96° C. and on analysis is found to contain 3.8% of sulphur. (C<sub>46</sub>H<sub>57</sub>N<sub>3</sub>SO<sub>10</sub> requires 3.8% of sulphur.)

The 4-(4-methoxybenzoylacetamido)-2:5-diethoxyaniline used in the above example is prepared as follows:

A mixture of 40 parts of 4-(4-methoxybenzoylacetamido)-2:5-diethoxy nitrobenzene, 800 parts of ethyl alcohol and Raney nickel catalyst is heated with hydro-

A solution of 45 parts of anisoylacetic ester in 70 parts of xylene is added over 30 minutes to a refluxing mixture of 30.7 parts of 4-nitro-2:5-diethoxyaniline, 350 parts of xylene and 10 parts of pyridine.

The mixture is then distilled until 130 parts of distillate

## EXAMPLE 9

2-carboxy-N-{3-[5-chloro-4-methyl-2-hydroxyphenyl]aminocarbonylphenyl}benzamide-4-N'-(4-dodecylphenyl)sulphonamide



has been collected, the mixture is then refluxed for a further 4 hours. After standing for 15 hours the mixture is diluted with 300 parts of methanol, cooled in ice and the precipitated solid collected by filtration. The 40 parts of 4-(4-methoxybenzoylacetamido)nitrobenzene are obtained as a pale yellow needle crystal melting at 197-198°C.

## EXAMPLE 7

2-carboxy-N-[4-(methoxybenzoylacetamido)phenyl]benzamide-4-N'-(4-dodecylphenyl)sulphonamide



In place of the 8.05 parts of N-(β-aminoethyl)-1-hydroxy-2-naphthamide used in Example 3 there are used 9.94 parts of 4-(4-methoxybenzoylacetamido)aniline. The product obtained is heated with 60 parts of methanol, cooled and filtered. The 11.9 parts of 2-carboxy-N-[4-(4-methoxybenzoylacetamido)phenyl]benzamide-4-N'-(4-dodecylphenyl)sulphonamide are obtained as a solid

15 In place of the 8.05 parts of N-(β-aminoethyl)-1-hydroxy-2-naphthamide used in Example 3 there are used 9.65 parts of 3-amino-N-(5-chloro-4-methyl-2-hydroxyphenyl)benzamide. The product is isolated by pouring into an excess of petroleum ether. The 19.6 parts of 2-carboxy-N-[3-[5-chloro-4-methyl-2-hydroxyphenyl]aminocarbonylphenyl]benzamide-4-N'-(4-dodecylphenyl)sulphonamide are obtained as a solid melting at 210-213°C. and on analysis is found to contain 63.7% of carbon, 5.7% of hydrogen, 5.7% of nitrogen and

20 4.4% of sulphur. ( $C_{40}H_{46}N_3ClO_7$  requires 64.3% of carbon, 6.2% of hydrogen, 5.6% of nitrogen and 4.4% of sulphur.)

## EXAMPLE 10

35 N-[4[N-(1-phenyl-5-pyrazolonyl-3)-aminoacetyl]phenyl]phthalimide-4-N'-(4-dodecylphenyl)sulphonamide



melting at 189-190°C. and on analysis is found to contain 66.5% of carbon, 6.5% of hydrogen, 5.6% of nitrogen and 4.3% of sulphur. ( $C_{42}H_{49}N_3SO_8$  requires 66.8% of carbon, 6.5% of hydrogen, 5.6% of nitrogen and 4.2% of sulphur.)

## EXAMPLE 8

N-(4-methoxybenzoylacetamido)phenylphthalimide-4-N'-(4-dodecylphenyl)sulphonamide



A mixture of 9.94 parts of 4-(4-methoxybenzoylacetamido)aniline, 16.45 parts of phthalic anhydride-4-N-(4-dodecylphenyl)sulphonamide and 350 parts of glacial acetic acid is heated under reflux for 2 hours. After cooling the solid is filtered off and recrystallised from 320 parts of ethyl alcohol. The 12.6 parts of N-(4-methoxybenzoylacetamido)phenylphthalimide-4-N'-(4-dodecylphenyl)sulphonamide are obtained as a solid melting at 170-174°C. and on analysis is found to contain 68.4% of carbon, 6.6% of hydrogen and 5.7% of nitrogen.

45 In place of the 9.94 parts of 4-(4-methoxybenzoylacetamido)aniline used in Example 8 there are used 10.8 parts of 1-phenyl-3-(4-aminophenylacetyl)pyrazolone, the preparation of which is described in Example 26 of British patent specification No. 830,797. The product is recrystallised from glacial acetic acid.

50 The 11.2 parts of N-[4[N-(1-phenyl-5-pyrazolonyl-3)-aminoacetyl]phenyl]phthalimide-4-N'-(4-dodecyl-

phenyl)sulphonamide are obtained as a solid melting at 228-231°C. and on analysis is found to contain 67.4% of carbon, 6.4% of hydrogen, 9.0% of nitrogen and 4.5% of sulphur. ( $C_{43}H_{47}N_5O_6S$  requires 67.8% of carbon, 6.2% of hydrogen, 9.2% of nitrogen and 4.2% of sulphur.)

## EXAMPLE 11

2-carboxy-N-[4-(3-phenylamino-5-pyrazolonyl-1-)phenylbenzamide-4-N'-(4-dodecylphenyl)sulphonamide



( $C_{42}H_{47}O_7N_3S$  requires 68.4% of carbon, 6.4% of hydrogen and 7.5% of nitrogen.)

75 In place of the 8.05 parts of N-(β-aminoethyl)-1-hydroxy-2-naphthamide used in Example 3 there are used

9.31 parts of 1-(3-aminophenyl)-3-anilino-5-pyrazolone. The product is recrystallised from ethyl alcohol. The 2-carboxy - N-[4-(3-phenylamino-5-pyrazolonyl-1)-phenyl] benzamide-4-(4-dodecylphenyl)sulphonamide is obtained as a solid melting at 155-157° C. and on analysis is found to contain 66.7% of carbon, 6.5% of hydrogen, 9.5% of nitrogen and 4.5% of sulphur. ( $C_{41}H_{47}N_5SO_6$  requires 66.7% of carbon, 6.4% of hydrogen, 9.5% of nitrogen and 4.3% of sulphur.)

## EXAMPLE 12

2-carboxy-N-[4-methoxy-3-(1-phenyl - 5 - pyrazolonyl-3-) aminophenyl]benzamide - 4 - N' - (4 - dodecylphenyl) sulphonamide



In place of the 8.05 parts of N-( $\beta$ -aminoethyl)-1-hydroxy-2-naphthamide used in Example 3 there are used 10.36 parts of 1-phenyl-3-(5-amino-2-methoxy)anilino-5-pyrazolone. The 11.2 parts of 2-carboxy-N-[3-methoxy-4-(1-phenyl - 5 - pyrazolonyl-3-) aminophenyl]benzamide-4-N'-(4-dodecylphenyl)sulphonamide are obtained as a solid melting at 216-219° C. and on analysis is found to contain 65.2% of carbon, 6.1% of hydrogen, 9.1% of nitrogen and 4.6% of sulphur. ( $C_{42}H_{49}N_5O_7$  requires 65.7% of carbon, 6.4% of hydrogen, 9.1% of nitrogen and 4.2% of sulphur.)

The preparation of 1-phenyl-3-(5-amino-2-methoxy)anilino-5-pyrazolone used in the above example is described in Example 32 of British Specification No. 956,261.

## EXAMPLE 13

2-carboxy-N-[ $\beta$ (1-hydroxy-2-naphthamido)ethyl] benzamide-4-N'n-octadecylsulphonamide



A mixture of 8.05 parts of N-( $\beta$ -aminoethyl)-1-hydroxy-2-naphthamide, 16.76 parts of phthalic anhydride-4-N-n-octadecylsulphonamide and 280 parts of ethyl acetate is heated under reflux for 2 hours. After cooling the solid reaction product is collected by filtration and re-

to dryness. To the residue is added 600 parts of acetyl chloride and the mixture heated under reflux for  $\frac{1}{2}$  hour. After filtering hot the solution is cooled to crystallise, the product collected by filtration and recrystallised from ethyl acetate. The 19 parts of phthalic anhydride-4-N-n-octadecylsulphonamide is obtained as a colourless solid melting at 128-132° C. and on analysis is found to contain 63.8% of carbon, 8.5% of hydrogen and 3.1% of nitrogen. ( $C_{26}H_{41}NSO_8$  requires 65.1% of carbon, 8.6% of hydrogen and 2.9% of nitrogen.)

## EXAMPLE 14

2-carboxy-N-(5-chloro-4-methyl-2-hydroxyphenyl)benzamide-4-N'-(4-dodecylphenyl)sulphonamide



9.14 parts of phthalic anhydride-4-N-(4-dodecylphenyl)sulphonamide, 2.8 parts of 2-amino-4-chloro-5-methylphenol and 100 parts by volume of dry ethyl acetate are heated at 60° for 0.75 hour. The mixture is cooled and then evaporated to a low bulk. The residue is taken up in methanol, and the insoluble material is filtered off. The methanol solution is evaporated at low temperature and the residue dissolved in sodium carbonate solution. The solution is filtered and the filtrate acidified with hydrochloric acid. The precipitate is filtered off, washed with water and dried at room temperature. The 8.8 parts of 2-carboxy-N-(5-chloro-4-methyl-2-hydroxyphenyl)benzamide-4-N'-(4-dodecylphenyl)sulphonamide are obtained as a solid melting at 145-148° C. On analysis, this compound is found to contain 4.3% of nitrogen and 4.7% of sulphur. ( $C_{33}H_{41}ClN_2O_6S$  requires 4.6% of nitrogen and 5.1% of sulphur.)

## EXAMPLE 15

2-carboxy-N-[2-{ $\beta$ (1-hydroxy-2-naphthamido)ethyl}phenyl]benzamide-4-N'-(4-dodecylphenyl)sulphonamide



9.14 parts of phthalic anhydride-4-N-(4-dodecylphenyl)sulphonamide, 6.2 parts of 2-( $\alpha$ -amino- $\beta$ -phenylethyl)-1-hydroxynaphthamide as described in United States patent specification 3,002,836 to Eastman Kodak Company, and 100 parts by volume of dry ethyl acetate are heated at 60° for 0.75 hour. The mixture is cooled and evaporated to dryness at low temperature. The product is dissolved out of the residue with methanol insoluble material being filtered off. The filtrate is evaporated to dryness and the residue dissolved in the theoretical quantity of sodium carbonate solution. This solution is filtered hot and after cooling, the colour coupler is obtained by acidifying with hydrochloric acid. The solid is filtered off and washed with water and dried at room temperature.

crystallised from ethyl acetate. The 7.0 parts of 2-carboxy - N - [ $\beta$ (1 - hydroxy-2-naphthamido)ethyl]benzamide-4-n-octadecylsulphonamide are obtained as a colourless solid melting at 225-226° C. and on analysis is found to contain 66.1% of carbon, 8.6% of hydrogen and 4.1% of sulphur. ( $C_{39}H_{55}N_3SO_7$  requires 66.1% of carbon, 7.8% of hydrogen and 4.5% of sulphur.)

The phthalic anhydride - 4-N-n-octadecylsulphonamide used in the above example may be prepared as follows:

A mixture of 26.9 parts of n-octadecylamine, 29.2 parts of phthalic acid-4-sulphonyl chloride, 8.2 parts of anhydrous sodium acetate and 400 parts of ethyl acetate is heated under reflux for 12 hours then evaporated down

11

The 10.1 parts of 2-carboxy-N-[2-( $\beta$ -(1-hydroxy-2-naphthamido)ethyl]phenyl]benzamide-4-N'-(4-dodecyl-phenyl)sulphonamide so obtained melted at 118-120°. On analysis, this compound is found to contain 68.0% of carbon, 6.2% of hydrogen, 5.5% of nitrogen and 3.9% of sulphur. ( $C_{45}H_{52}N_3O_7S$  requires 68.9% of carbon, 6.6% of hydrogen, 5.4% of nitrogen and 4.1% of sulphur.)

A photographic emulsion layer containing 2.81 parts of the colour coupler formulated by the method of Example 3 gives a cyan dye image with light absorption maximum at 690  $\mu\text{m}$ .

**EXAMPLE 16**

**2-carboxy-N-[6-(1-hydroxy-2-naphthamido)hexyl]benzamide-4-N'-(4-dodecylphenyl)sulphonamide**



6.5 parts of phthalic anhydride-4-N-(4-dodecylphenyl)sulphonamide, 5.0 parts of 1-(1-hydroxy-2-naphthamide)-6-aminohexane and 100 parts by volume of dry ethyl acetate are heated under reflux for 0.75 hour. The solution is evaporated to dryness at a low temperature and then dissolved in 2 normal sodium carbonate solution. Any insoluble material is filtered off and the filtrate is acidified with hydrochloric acid. The precipitated solid is filtered off, washed with water and dried at room temperature.

The 6.0 parts of 2-carboxy-N-[6-(1-hydroxy-2-naphthamido)hexyl]benzamide-4 - N' - (4 - dodecylphenyl)sulphonamide so obtained is a solid melting at 117-120°. On analysis this compound is found to contain 67.0% of carbon, 6.9% of hydrogen, 5.6% of nitrogen and 3.9% of sulphur. ( $C_{43}H_{55}N_3O_7S$  requires 68.2% of carbon, 7.3% of hydrogen, 5.6% of nitrogen and 4.2% of sulphur.)

**EXAMPLE 17**

2-carboxy-N-[2-{ $\beta$ -(4-chloro-1-hydroxy-2-naphthamido)ethyl}phenyl]benzamide-4-N'-(4-dodecylphenyl)sulphonamide



8.0 parts of phthalic anhydride-4-N-(4-dodecylphenyl)sulphonamide, 5.95 parts of 2-(o-amino- $\beta$ -phenylethyl)-1-hydroxy-4-chloronaphthamide and 100 parts of dry ethyl acetate are heated under reflux for 0.75 hour. The mixture is cooled and any precipitated material is filtered off and the filtrate evaporated to dryness. The residue is dissolved in sodium carbonate solution and the solution is filtered. The filtrate is made acid with hydrochloric acid and the product filtered off, washed with water and then dried. The 6.7 parts of 2-carboxy-N-[2-{ $\beta$ -(4-chloro-1-hydroxy-2-naphthamido)ethyl}phenyl]benzamide-4-N'-(4-dodecylphenyl)sulphonamide so obtained melted at 186°.

12

with decomposition. On analysis it is found to contain 4.6% of chlorine, 4.9% of nitrogen and 4.2% of sulphur. ( $C_{45}H_{51}ClN_3O_7S$  requires 4.4% of chlorine, 5.2% of nitrogen and 3.9% of sulphur.)

5 A photographic emulsion layer containing 2.93 parts of the colour coupler formulated by the method of Example 3 gives a cyan dye image with light absorption maximum at 685 m $\mu$ .

### EXAMPLE 18

## 2-carboxy-N-[3-(4-methoxybenzoylacetamido)-4-methoxyphenyl]benzamide-4-N'-n-octadecylsulphonamide



20 In place of the 8.05 parts of  $N$ -( $\beta$ -aminoethyl)-1-hydroxy-2-naphthamide used in Example 13 there are used 10.85 parts of 4-methoxy-3-(4-methoxybenzoyl acetamido)aniline. The product is recrystallised from 140 parts of ethyl alcohol. The 2-carboxy- $N$ -[3-(4-methoxybenzoylacetamido)-4-methoxyphenyl]benzamide - 4- $N'$ -n-octadecylsulphonamide is obtained as a solid melting at 138-140° C.

I claim as my invention:

1. A color coupler which is a compound selected from the group consisting of compounds of the formula:



40 and corresponding cyclised compounds of the formula:



wherein R is a member selected from the group consisting of alkyl and alkyl-substituted phenyl, wherein the alkyl radical and the alkyl substituent contain from 12 to 18 carbon atoms, and B is the residue of a compound RNH, which is selected from the group consisting of

$$(1) \quad X-B_1-CO-CH=CO-NH-B_2-Y$$



and (3) primary amino compounds selected from the group consisting of N-( $\beta$ -aminoethyl)-1-hydroxy-2-naphthamide, N-( $\beta$ -aminoethyl)-4-chlor-1-hydroxy-2-naphthamide, 3-amino-N-(5-chloro-4-methyl-2-hydroxy-phenyl)benzamide, 2-amino-4-chloro-5-methylphenol, 2-(o-amino- $\beta$ -phenylethyl)-1-hydroxynaphthamide, 1-(1-hydroxy-2-naphthamide)-6-aminohexane, and 2-(o-amino- $\beta$ -phenylethyl)-1-hydroxy-4-chloronaphthamide,

- wherein  $R_1$  and  $R_2$  are independently selected from the group consisting of phenyl, methoxyphenyl, di-carbomethoxyphenyl, and diethoxyphenyl,  
 $R_3$  is phenyl,  
one of X and Y is  $-NH_2$  and the other is H,  
 $X_1$  is  $-NH_2$  and  $Y_1$  is anilino or  $X_1$  is H and  $Y_1$  is  $-NH_2$ , aminophenylacetyl amino, or (2-methoxy-5-amino)anilino.  
2. A compound according to claim 1 wherein R represents dodecyl phenyl.  
3. A compound according to claim 1 wherein R represents stearyl.  
4. A compound according to claim 1 wherein B represents 1-phenyl-5-pyrazolonyl-1.  
5. A compound according to claim 1 wherein B is the residue of a compound  $BNH_2$  which is selected from the group consisting of N-( $\beta$ -aminoethyl)-1-hydroxy-2-naphthamide, N - ( $\beta$  - aminoethyl) - 4 - chloro - 1 - hydroxy - 2 - naphthamide, 2 - (o - amino -  $\beta$  - phenylethyl) - 1 - hydroxynaphthamide, 1 - (1 - hydroxy - 2 - naphthamide)-6-aminohexane, and 2-(o-amino- $\beta$ -phenylethyl)-1-hydroxy-4-chloronaphthamide.  
20 6. A compound according to claim 1 wherein B represents paramethoxy benzoyl acet.

## References Cited

## UNITED STATES PATENTS

|           |        |                       |           |
|-----------|--------|-----------------------|-----------|
| 2,083,216 | 6/1937 | Benade et al. -----   | 260-310   |
| 2,710,803 | 6/1955 | Salminen et al. ----- | 260-310   |
| 2,837,557 | 6/1958 | Lynn -----            | 260-465.4 |
| 2,878,263 | 5/1959 | Oroshnik -----        | 260-310   |
| 2,905,694 | 9/1959 | Pinson -----          | 260-310   |
| 2,933,391 | 4/1960 | Feniak et al. -----   | 96-100    |
| 2,983,608 | 5/1961 | Beavers -----         | 96-100    |
| 3,034,891 | 5/1962 | Burgardt et al. ----- | 260-465   |
| 3,148,178 | 9/1964 | Wallace et al. -----  | 260-326   |

## OTHER REFERENCES

Cram et al.: Organic Chemistry, McGraw-Hill Book Co., Inc., New York, 1959, p. 384.

ALEX MAZEL, *Primary Examiner.*

NORMAN G. TORCHIN, HENRY R. JILES,  
NICHOLAS S. RIZZO, *Examiners.*

M. O'BRIEN, J. T. BROWN, *Assistant Examiners.*